

Feb. 13, 1951

M. P. KULP

2,541,165

METHOD FOR PRODUCING GLOBULAR ARTICLES

Original Filed Feb. 15, 1947



INVENTOR.  
MAURICE P. KULP  
BY

*Thomas R. Kelly  
Attorney*

## UNITED STATES PATENT OFFICE

2,541,165

## METHOD FOR PRODUCING GLOBULAR ARTICLES

Maurice P. Kulp, Linwood, Pa., assignor to American Viscose Corporation, Wilmington, Del., a corporation of Delaware

Original application February 15, 1947, Serial No. 728,788. Divided and this application February 4, 1948, Serial No. 6,143

7 Claims. (Cl. 18—48)

1

This invention relates to the production of globular particles of regenerated cellulose, particularly from viscose. This application is a division of copending application Serial No. 728,788, filed February 15, 1947.

Methods that have heretofore been employed for making globular particles from viscose resulted generally in products which not only were far from sphericity but were marred by numerous checks and fissures resulting from the inability to prevent the development of gases within the globules during regeneration and the inability to prevent irregular shrinkage during regeneration, subsequent wet processing, and drying of the globules.

In accordance with the present invention these difficulties are substantially completely avoided. This is accomplished by allowing droplets of viscose to form in a gaseous atmosphere and fall into a substantially non-regenerating bath from a height which is sufficient to allow the droplet to assume a substantially spherical shape prior to entering the bath. The height required depends upon the size of droplet which can be varied by varying the size of orifice, the temperature of the viscose, or the pressure exerted on the viscose passing through the orifice. A droplet of a size which forms a particle of  $\frac{1}{8}$  inch diameter requires a drop of at least 6 feet, while smaller droplets will require less drop and larger ones a greater drop to allow the surface tension sufficient time to overcome the non-sphericity of a droplet of viscose having a viscosity of about 40 (ball fall). After a short period in the non-regenerating bath (between  $\frac{1}{2}$  and 10 minutes), the superficially coagulated structure is introduced into a heated liquid of non-solvent, non-softening and non-acid character in which coagulation and regeneration of the globules are completed. Suitable liquids for this purpose are hot aqueous salt solutions at a temperature below the boiling point of water.

After the globules are taken from the heated liquid, the by-products of regeneration, such as alkaline and sulfur compounds, are in a water-soluble state and are merely leached out by introducing the globules into water, preferably hot, for the desired period of time. Thereafter, the globules may be dried or, before drying, they may be soaked in a plasticizer, such as glycerine, when a softened product is desired. Shrinkage to any substantial extent can only occur during the drying step of this procedure since the contact of the globules with acid is restricted to a minimum and the globules are maintained in

water-swelled condition thereafter until the drying stage. It has been found that the shrinkage that occurs during the drying of the globules formed in accordance with the procedure of this invention is remarkably uniform in character and substantially iso-tropic so that they undergo little change in their original shape other than a diminution in size during the drying.

The original shape of the globules formed depends upon the height from which the viscose droplets are allowed to fall into the acid bath. If dropping heights are used which are considerably greater (more than about 20% greater) than the minimum needed to obtain sphericity, the size of the droplet falling from the dropping orifice or jet does not determine the ultimate size of the product as in such cases, they tend to disrupt into numerous smaller particles which may have various sizes, and, in the extreme of conditions, a powdered product results.

The sole figure of the drawing illustrates one arrangement for executing the invention.

As shown in the drawing, the viscose solution in a vessel 2 which may be provided with a plunger 3 for exerting pressure thereon passes through a dropping tube terminating in an orifice 4. A receptacle 5 for the coagulating bath is arranged beneath the hopper to receive the droplets and preferably has a sloped bottom 6 to facilitate removal of the particles roughly in their order of production.

The bath in the receptacle 5 may advantageously be an aqueous solution containing 3 to 6% acetic acid and 16 to 20% sodium sulfate at 40 to 50° C., and the particles are allowed sufficient contact therewith to form a thin coagulated skin thereon. Then they are removed and placed in a 20% sodium sulfate solution in water at 60° to 70° C. or up to the boiling point of water. This bath is agitated and the treatment is carried on for about an hour. Finally, the pellets or granules are removed from the salt bath and introduced into a leaching vessel in which they are subjected for 8 to 12 hours or longer to a flow of hot water at 60° to 70° C. or higher. This completes the purification of the pellets while substantially preventing any irregular shrinkage. The particles may remain in this bath an indefinite period or they may be stored in cold or hot water for an indefinite period before ultimate drying. However, if convenient, drying may be performed directly after the leaching period of 8 to 12 hours mentioned. Preferably, the humidity is controlled to prevent irregular shrinkage.

The final products which may be of any size up to the order of  $\frac{1}{3}$  inch in diameter approach true sphericity and are substantially free of checks, fissures, bubbles, creases and wrinkles. The unplasticized products are hard and have a high dielectric constant. Because of this characteristic and the fact that the products are highly resistant to hydrocarbon oils they may be used in conjunction with such oils for cooling electrical equipment, such as transformers. The unplasticized products may be coated with moistureproofing and chemically resistant compositions where their use would involve prolonged contact with moisture, acids, alkalies, or other corrosive fluids. The plasticized products are of use where flexibility is desirable.

It is to be understood that changes and variations may be made without departing from the spirit and scope of the invention as defined by the appended claims.

I claim:

1. The method of making granular particles comprising regenerated cellulose comprising the steps of allowing droplets of viscose to fall into a substantially non-regenerating aqueous salt-containing dilute acid bath, removing the formed granules of viscose from the bath after a superficial coagulation thereof, and introducing the superficially coagulated granules into a heated non-acid aqueous salt-containing bath incapable of softening the granules and having a temperature of at least 60° C.

2. The method of making granular particles comprising regenerated cellulose comprising the steps of allowing droplets of viscose to fall through air into a substantially non-regenerating salt-containing bath containing acetic acid, removing the formed granules of viscose from the bath after a thin skin has been formed thereon, introducing the superficially coagulated granules into a heated non-acid aqueous salt-containing bath incapable of softening the granules and having a temperature of at least 60° C., and then leaching the granules.

3. The method of making granular particles comprising regenerated cellulose comprising the steps of allowing droplets of viscose to fall through the air from a sufficient height into a

substantially non-regenerating salt-containing bath containing acetic acid to cause the droplets to assume a spherical shape before entering the bath, removing the formed granules of viscose from the bath after a thin skin has been formed thereon, introducing the superficially coagulated granules into a heated non-acid aqueous salt-containing bath incapable of softening the granules and having a temperature of at least 60° C.

4. The method of making granular particles comprising regenerated cellulose comprising the steps of allowing droplets of viscose to fall into a non-regenerating bath consisting of sodium sulfate, acetic acid, and water, removing the formed granules of viscose from the bath after a thin skin has been formed thereon, and introducing the superficially coagulated granules into a heated aqueous sodium sulfate solution having a temperature of at least 60° C.

5. The method of making regenerated cellulose globules approaching sphericity in shape comprising the steps of allowing viscose to fall in the form of individual drops into a non-regenerating bath consisting of 10 to 20% sodium sulfate, 3 to 6% acetic acid, and water, removing the formed globules from the bath after a thin skin has been formed thereon, introducing the superficially coagulated globules into a heated bath consisting of sodium sulfate and water having a temperature of at least 60° C.

6. The method of claim 5 followed by the step of leaching the particles in hot water, and drying them.

7. The method of claim 6 in which the first bath is at about 40° to 50° C. and the subsequent baths are at temperatures of 60° to 99° C.

MAURICE P. KULP.

REFERENCES CITED

The following references are of record in the file of this patent:

UNITED STATES PATENTS

| Number    | Name          | Date          |
|-----------|---------------|---------------|
| 2,249,745 | Church et al. | July 22, 1941 |
| 2,413,123 | Underwood     | Dec. 24, 1946 |
| 2,465,343 | Battista      | Mar. 29, 1949 |